

Nov. 28, 1950

P. H. CARNELL

2,531,723

PROCESS OF IMPROVING LUBRICATING OILS BY TREATING  
WITH HYDROFLUORIC ACID AND SILVER FLUORIDE

Filed Dec. 15, 1947



INVENTOR.  
P. H. CARNELL

BY

*Hudson & Young*

ATTORNEYS

## UNITED STATES PATENT OFFICE

2,531,723

PROCESS OF IMPROVING LUBRICATING  
OILS BY TREATING WITH HYDRO-  
FLUORIC ACID AND SILVER FLUORIDEPaul H. Carnell, Alma, Mich., assignor to Phillips  
Petroleum Company, a corporation of Delaware

Application December 15, 1947, Serial No. 791,803

5 Claims. (Cl. 196—39)

1

This invention relates to the treatment of lubricating oils to improve their properties. In one of its more specific aspects, it relates to a treatment of a lubricating oil which improves its viscosity index.

I have discovered that treatment of a lubricating oil with substantially anhydrous hydrofluoric acid, a low-boiling hydrocarbon, such as isopentane, and silver fluoride will improve the viscosity index of the oil.

Lubricating oil referred to herein, includes all such products and their base stocks which have a viscosity within the range of about 32 S. U. S. (Saybolt Universal seconds) at 210° F. to about 350 S. U. S., at 210° F., and as are usually understood to be covered by this term by those skilled in the art. It includes lubricating oil stocks, such as, paraffin-base stock, naphthene-base stock, synthetic-base stock, and mixed-base stock, which are refined for use as engine lubricants.

The hydrofluoric acid and silver fluoride used in the practice of this invention, may be of the quality of the commercial products. The hydrofluoric acid, referred to as substantially anhydrous hydrofluoric acid, may contain small amounts of sulfur dioxide (usually less than 1 weight per cent), water, and other impurities.

I have found that silver fluoride, when used in conjunction with hydrofluoric acid and a low-boiling hydrocarbon for the treatment of lubricating oils, is unexpectedly effective in producing improved lubricating oils. In particular, when a lubricating oil is treated with a mixture of hydrofluoric acid, a low-boiling hydrocarbon, such as isopentane, and silver fluoride, a pronounced improvement in the viscosity index of the oil is obtained. However, if silver chloride is substituted for silver fluoride in the above-mentioned mixture, the viscosity index of the oil is not improved. Likewise, when lead fluoride is substituted for silver fluoride in the above treatment there is no improvement in viscosity index.

The effectiveness of a given promoter, in this hydrofluoric acid process for treating lubricating oils, appears to be in part, a matter of its solubility in hydrofluoric acid. Thus, silver fluoride is an active promoter and is soluble in hydrofluoric acid, whereas silver chloride and lead fluoride are inactive and relatively insoluble in hydrofluoric acid.

An object of the present invention is to provide a novel and improved method for improving lubricating oils. Another object is to provide a method for improving natural lubricating oils. Another object is to provide a method for improving synthetic lubricating oils. Another object is to provide a method for improving mixed-base lubricating oils. Another object is to provide a method for improving the viscosity index of lubricating oils. Other objects and advantages

2

of this invention will become apparent from the accompanying disclosure and discussion.

Broadly speaking, my invention comprises a process for improving lubricating oil by contacting the lubricating oil with substantially anhydrous hydrofluoric acid, and silver fluoride. In a preferred embodiment, a low-boiling hydrocarbon is also included in the reaction mixture.

Generally speaking, lubricating oil, substantially anhydrous hydrofluoric acid, a low-boiling liquid hydrocarbon, such as isopentane, and finely divided silver fluoride are introduced to a contact chamber. Usually satisfactory results can be obtained with this process if temperatures within the range of about 20 to about 40° C. and pressures of about atmospheric pressure are used. However, with particular oils, it may be desirable to use elevated temperatures as high as 300° C., and superatmospheric pressures. The contact time will generally vary from about 20 to about 120 minutes, depending on the type of agitation used, degree of oil improvement desired, etc. Suitable volume ratios of oil to hydrofluoric acid to light hydrocarbon are about 1:3:5 to about 5:3:1, but preferably about 1:1:1. The weight of silver fluoride required is about 1 to about 10 weight per cent of the acid present.

A better understanding of my invention may be had by referring to the accompanying schematic flow diagram of a preferred embodiment.

Referring to the attached diagram, a low-boiling hydrocarbon, such as isopentane, hydrofluoric acid and silver fluoride, and lubricating oil are charged to contactor 10 through lines 11, 12, and 13 respectively, where they are agitated the required length of time, usually for about 20 to about 120 minutes, at a moderate or elevated temperature. The treated mixture is passed through line 14 to settler 16 where it is separated into an upper layer consisting of lubricating oil and hydrocarbons boiling below the lubricating oil range, part of which are formed by chemical reaction in contactor 10, and possibly some suspended silver fluoride; and a lower layer consisting of hydrofluoric acid, silver fluoride, and acid soluble organic materials. The lower layer from settler 16 is passed through line 17 to fractionator 18, and the upper layer is passed through line 19 to fractionator 20. Hydrofluoric acid from fractionator 18 is removed through line 21 and recycled to contactor 10. The silver fluoride-acid soluble oil mixture from the kettle of fractionator 18 is passed through line 21 to recovery unit 22. Generally, the silver fluoride may be recovered from the acid-soluble oil by filtration. However, when the acid soluble oil is unusually heavy, it may be desirable to add a suitable organic solvent before filtering, which is introduced through line 25. The recovered silver fluoride, to which has been added hydrofluoric acid, is recycled from

unit 22 to contactor 10 as a slurry, through line 23.

The oil and solvent from recovery unit 22 are passed through line 24 to recovery unit 26 where the solvent is removed for recycle through lines 27, 25, and 21 to unit 22. The oil from unit 26 is recovered through line 28 as a by-product of the process. The low-boiling hydrocarbon from fractionator 20 is recycled to contactor 10 through line 29. Other relatively light hydrocarbons from fractionator 20, distilling below the lubricating oil boiling range, may be recycled to contactor 10 through line 29 or withdrawn as by-products of the process through line 30. Lubricating oil from the kettle of fractionator 29 is withdrawn through line 31 as the product of the process. If desired, this product may be passed to the silver fluoride and oil-solvent recovery units through line 32 to remove any small amounts of suspended silver fluoride. The recovery of silver fluoride from the product lubricating oil may be carried out in the same apparatus as that used in the processing of the acid soluble oil for silver fluoride recovery. The treatment of the two must be separate, however, to avoid contamination of the product oil with acid soluble oil.

Various additional valves, pumps, and other conventional equipment necessary for the successful practice of this invention will be familiar to one skilled in the art and have been omitted from this schematic drawing for the sake of clarity.

To further illustrate some of the many aspects of this invention, the following specific example is given.

A 4½-liter steel bomb was charged with hydrofluoric acid, isopentane, a mixed-base lubricating oil, and when desired, a metallic halide. The bomb was clamped to a platform rocker and agitated for 60 minutes at room temperature. The contents of the bomb were allowed to settle for one hour, and the acid layer was then withdrawn. The hydrocarbon layer was caustic washed, filtered, and topped to the initial boiling point of the untreated oil in a vacuum fractionating column to remove light ends. The following data were obtained:

| Run                             | Charge<br>Oil <sup>1</sup> | 1                       | 2                       | 3                       | 4     |
|---------------------------------|----------------------------|-------------------------|-------------------------|-------------------------|-------|
| Oil, ml.                        |                            | 1,000                   | 1,000                   | 1,000                   | 1,000 |
| HF, ml.                         |                            | 1,000                   | 1,000                   | 1,000                   | 1,000 |
| Isopentane, ml.                 |                            | 1,000                   | 1,000                   | 1,000                   | 1,000 |
| Halide.                         | None <sup>2</sup>          | ( <sup>1</sup> )<br>100 | ( <sup>2</sup> )<br>100 | ( <sup>3</sup> )<br>100 |       |
| Halide, grams.                  |                            |                         |                         |                         |       |
| Product Oil.                    |                            |                         |                         |                         |       |
| Viscosity, 100°F, S. U. S.      | 388.3                      | 374.9                   | 318.6                   | 372.2                   | 366.3 |
| Viscosity, 210°F, S. U. S.      | 55.62                      | 55.17                   | 53.63                   | 54.79                   | 54.42 |
| Viscosity index (Dean & Davis). | 85                         | 87                      | 99                      | 86                      | 85    |
| A. P. I. gravity                | 28.4                       | 28.6                    | 31.6                    | 28.7                    | 28.7  |

<sup>1</sup> Silver fluoride.

<sup>2</sup> Silver chloride.

<sup>3</sup> Lead fluoride.

The data of run 2 show that when a given lubricating oil is treated with a mixture of hydrofluoric acid, isopentane, and silver fluoride, at room temperature, the viscosity index of the product oil is about 12 units higher than the viscosity index of the oil treated with a hydrofluoric acid-isopentane mixture in the absence of silver fluoride. The data from runs 3 and 4 show less improvement in the oil than is obtained by leaving a metallic halide out of the treatment altogether, as shown in run 1.

Although this invention has been described and

exemplified in terms of its preferred modification, it is understood that various changes may be made without departing from the spirit of the process as disclosed and expressed in the claims.

I claim:

1. A process for improving the viscosity index of a lubricating oil which comprises treating a lubricating oil with a reagent consisting of a mixture of substantially anhydrous hydrofluoric acid and silver fluoride.

2. The process of producing a lubricating oil of improved viscosity index which comprises treating a lubricating oil with a reagent consisting of a mixture of substantially anhydrous hydrofluoric acid and solid silver fluoride in the presence of a low-boiling liquid hydrocarbon diluent, said treatment taking place at a temperature in the range of about 20 to about 300° C., at a moderate to high pressure, and for a period of time in the range of about 20 to about 120 minutes, and recovering an improved lubricating oil.

3. The process of manufacturing a lubricating oil of improved viscosity index, which comprises treating a lubricating oil with a reagent consisting of a mixture of substantially anhydrous hydrofluoric acid and finely divided silver fluoride in the presence of a low-boiling liquid hydrocarbon diluent, the volume ratio of oil to hydrofluoric acid to light hydrocarbon being in the range of about 1:3:5 to about 5:3:1, the weight of silver fluoride to hydrofluoric acid being in the range of about 1 to about 10 weight per cent of the acid, said treatment of lubricating oil taking place at a temperature in the range of about 20 to about 300° C., at a moderate to high pressure, and for a period of time within the range of about 20 to about 120 minutes, and recovering an improved lubricating oil as a product of the process.

4. The process of manufacturing a lubricating oil of improved viscosity index, which comprises treating a lubricating oil with a reagent consisting of a mixture of substantially anhydrous hydrofluoric acid and solid finely divided silver fluoride in the presence of isopentane diluent, the ratio of oil to hydrofluoric acid to isopentane being in the range of about 1:1:1, the weight of silver fluoride to hydrofluoric acid being in the range of about 1 to about 10 weight per cent of the acid, said treatment of lubricating oil taking place at a temperature in the range of about 20 to about 40° C., at about atmospheric pressure, and for a period of time within the range of about 20 to about 120 minutes, and recovering an oil of improved viscosity index as a product of the process.

5. A process according to claim 1 wherein a low-boiling hydrocarbon diluent is used in admixture with said oil and reagent.

PAUL H. CARNELL.

#### REFERENCES CITED

The following references are of record in the file of this patent:

#### UNITED STATES PATENTS

| Number       | Name     | Date          |
|--------------|----------|---------------|
| 2,366,743    | Matuszak | Jan. 9, 1945  |
| 2,375,675    | Matuszak | May 8, 1945   |
| 70 2,378,762 | Frey     | June 19, 1945 |

#### FOREIGN PATENTS

| Number  | Country       | Date         |
|---------|---------------|--------------|
| 292,932 | Great Britain | May 23, 1929 |

**Certificate of Correction**

Patent No. 2,531,723

November 28, 1950

**PAUL H. CARNELL**

It is hereby certified that error appears in the printed specification of the above numbered patent requiring correction as follows:

Column 4, lines 15 and 44, strike out the word "solid"; line 26, same column, strike out "finely divided";

and that the said Letters Patent should be read as corrected above, so that the same may conform to the record of the case in the Patent Office.

Signed and sealed this 1st day of May, A. D. 1951.

[**SEAL**]

**THOMAS F. MURPHY,**  
*Assistant Commissioner of Patents.*